

# UNITED STATES PATENT OFFICE.

HANS T. CLARKE, OF ROCHESTER, NEW YORK, ASSIGNOR TO EASTMAN KODAK COMPANY, OF ROCHESTER, NEW YORK, A CORPORATION OF NEW YORK.

## CELLULOSE-NITRATE COMPOSITION.

1,370,878.

Specification of Letters Patent.

Patented Mar. 8, 1921.

No Drawing.

Application filed March 17, 1919. Serial No. 283,228.

To all whom it may concern:

Be it known that I, HANS T. CLARKE, a subject of the King of Great Britain, residing at Rochester, in the county of Monroe 5 and State of New York, have invented certain new and useful Improvements in Cellulose-Nitrate Compositions, of which the following is a full, clear, and exact specification.

10 This invention relates to a new composition of matter and a method of making the same, in which cellulose nitrate is combined or mixed with other substances, so that the resulting product can be advantageously 15 used in the plastic and analogous arts, such, for instance, as sheet or film manufacture and varnish manufacture.

One object is to produce a composition which may be made into permanently trans- 20 parent, strong and flexible sheets or film of desired thinness that are substantially waterproof, are unaffected by ordinary photographic fluids and possess the desired properties of a support for sensitive photographic coatings. Another object of my invention is to produce a composition of matter capable of easy manipulation in the plastic and film making or varnish making arts; which will not injure or be injured by the 25 substances with which it is associated during manufacture, storage, or use. Still another object of my invention is to provide a process for compounding such composition of matter. Further objects will hereinafter 30 appear.

I have discovered that a composition of matter having the desirable qualities hereinabove enumerated can be obtained by mixing or compounding cellulose nitrate with 35 simple alkyl sulfones which are only slightly volatile or non-volatile at ordinary temperatures. By simple alkyl sulfones I mean substances of the type indicated by the following formulæ in which A and B represent alkyl groups:



50 There are noted, for example, normal diethyl sulfone, diisobutyl sulfone, dimethyl sulfone, diethyl sulfone, normal dipropyl sulfone, diisopropyl sulfone, diisoamyl sulfone, methyl ethyl sulfone, diheptyl sulfone

and ethylisoamyl sulfone. These may, of course, be mixed as well as used singly, and the degree of purity will depend upon the purposes to which the plastic composition is to be put. These substances vary as regards their boiling points, tendencies to volatilize, and solubilities with respect to water; and so are useful in varying ways in different branches of the plastic arts. These sulfones all have boiling points above 200° C. and are very stable. The latter property is particularly essential in the photographic art where the liberation of breakdown sulfur products might impair the light-sensitive coating. Their properties appear in various degrees in their homologues and derivatives. The compounding is best performed by using a solvent common to both the cellulose nitrate and the sulfone.

For flexible film and varnish manufac- 75 ture, the simple alkyl sulfone should be so nearly non-volatile that its loss during the desired life of the film will not be sufficient to make the latter unserviceable. They are less combustible than cellulose nitrate and 80 impart this quality to a very useful degree to the compound.

As a typical useful example of the dialkyl sulfones, which may be employed in exercising my invention, the normal dibutyl sulfone is selected. It is a white solid at ordinary temperatures and its boiling point is above 250° C., so that its volatility when compounded with nitrocellulose is practi- 85 cally nil. It is practically insoluble in wa- 90 ter and very stable.

In carrying out one illustration of my invention, I incorporate in 20 to 30 parts of an acetone and methyl alcohol mixture the following ingredients: cellulose nitrate 3 to 95 6 parts, (say, for instance, 5 parts) normal dibutyl sulfone  $\frac{1}{2}$  part to 10 parts. The acetone and methyl alcohol may be present in varying proportions, a two to one mixture being satisfactory. The ingredients are 100 mixed to form a homogeneous solution or flowable mass and are filtered if desired. High boiling auxiliary softeners may be added if desired, in small amounts, say  $\frac{1}{2}$  to 2 parts, such as higher aliphatic alcohols or their esters, like fusel oil, amyl acetate, butyl acetate, ethyl propionate, ethyl butyrate, etc.

The solution, either with or without the additional high boiling softener, is sufficiently thick and viscous to be properly flowed during sheet or film manufacture, the 5 acetone and methyl alcohol volatilizing, but not too rapidly to impair the product. The resulting film containing the cellulose nitrate and sulfone, together with the additional high boiling softener if the latter is 10 used, is very flexible, transparent, and uniform, so that it can be used for any usual or preferred purpose. It is practically waterproof and unaffected by ordinary photographic chemicals. The sulfones are so 15 stable that they do not in any appreciable degree liberate products which injure metal or other parts with which they come in contact during manufacture; and moreover they do not chemically react with or injure 20 the other bodies that are associated with them in the solution or the completed film.

While I have hereinabove disclosed certain compositions and processes by way of example, my invention is not limited thereto 25 nor to the proportions given therein, as the proportions may be varied from those given and equivalent substances may be substituted without departing from the principle of my invention as defined in the appended 30 claims.

Having thus described my invention, what I claim as new and desire to secure by Letters Patent is:

1. A transparent composition of matter comprising cellulose nitrate and a simple dialkyl sulfone.
2. A composition of matter comprising cellulose nitrate and a dibutyl sulfone.
3. A flowable film-forming composition 40 of matter comprising cellulose nitrate, a simple dialkyl sulfone, and a solvent common to both.
4. A composition of matter comprising

cellulose nitrate, a dibutyl sulfone, and a solvent common to both.

5. A flowable film-forming composition of matter comprising cellulose nitrate, a simple dialkyl sulfone and a solvent containing acetone and methyl alcohol.

6. A composition of matter comprising 50 cellulose nitrate, a dibutyl sulfone and a solvent containing acetone and methyl alcohol.

7. A composition of matter comprising cellulose nitrate, a simple dialkyl sulfone, a solvent common to both, and an organic body of only slight volatility which enhances the plasticity and flexibility of the composition.

8. A composition of matter comprising 60 acetone 10 to 20 parts, methyl alcohol 10 to 20 parts, cellulose nitrate 3 to 6 parts, dibutyl sulfone 1 to 10 parts.

9. As an article of manufacture, a tough 65 flexible sheet of deposited or flowed cellulose nitrate containing a simple dialkyl sulfone.

10. As an article of manufacture, a sheet 70 of deposited or flowed cellulose nitrate containing a dibutyl sulfone.

11. As an article of manufacture, a sheet 75 of deposited or flowed cellulose nitrate containing a simple dialkyl sulfone and an organic body of slight volatility which enhances the flexibility of the sheet.

12. The process of making a composition 80 of matter which consists in combining cellulose nitrate and a simple dialkyl sulfone in a solvent common to both.

13. The process of making a composition 85 of matter which consists in combining cellulose nitrate and a dibutyl sulfone by the use of a solvent containing acetone and methyl alcohol.

Signed at Rochester, New York, this 15th day of March 1919.

HANS T. CLARKE.